



US010794007B2

(12) **United States Patent**  
**Vogt et al.**

(10) **Patent No.:** **US 10,794,007 B2**  
(b4) **Date of Patent:** **\*Oct. 6, 2020**

(54) **LOTION TREATED THROUGH-AIR DRIED  
TISSUE**

(71) Applicant: **Kimberly-Clark Worldwide, Inc.**,  
Neenah, WI (US)

(72) Inventors: **Kevin Joseph Vogt**, Neenah, WI (US);  
**Jeffrey Dean Holz**, Sherwood, WI (US); **Mike Thomas Goulet**, Neenah, WI (US)

(73) Assignee: **KIMBERLY-CLARK WORLDWIDE, INC.**, Neenah, WI (US)

(\*) Notice: Subject to any disclaimer, the term of this patent is extended or adjusted under 35 U.S.C. 154(b) by 0 days.

This patent is subject to a terminal disclaimer.

(21) Appl. No.: **16/084,280**

(22) PCT Filed: **Mar. 21, 2017**

(86) PCT No.: **PCT/US2017/023325**

§ 371 (c)(1),  
(2) Date: **Sep. 12, 2018**

(87) PCT Pub. No.: **WO2017/165358**

PCT Pub. Date: **Sep. 28, 2017**

(65) **Prior Publication Data**

US 2019/0078262 A1 Mar. 14, 2019

**Related U.S. Application Data**

(60) Provisional application No. 62/313,066, filed on Mar. 24, 2016.

(51) **Int. Cl.**

**D21H 21/24** (2006.01)  
**D21H 17/07** (2006.01)  
**D21H 17/53** (2006.01)  
**D21H 19/24** (2006.01)  
**D21H 19/84** (2006.01)  
**D21H 27/00** (2006.01)  
**D21H 21/22** (2006.01)  
**A47K 10/16** (2006.01)

(52) **U.S. Cl.**

CPC ..... **D21H 21/24** (2013.01); **D21H 17/07** (2013.01); **D21H 17/53** (2013.01); **D21H 19/24** (2013.01); **D21H 19/84** (2013.01); **D21H 21/22** (2013.01); **D21H 27/00** (2013.01); **D21H 27/002** (2013.01); **D21H 27/004** (2013.01); **A47K 10/16** (2013.01)

(58) **Field of Classification Search**

CPC ..... D21H 27/002; D21H 17/53; D21H 21/14; D21H 27/00; D21H 17/06; D21H 17/07; D21H 17/36; D21H 19/24; D21H 19/84; D21H 23/22; D21H 27/004; A47K 10/16

See application file for complete search history.

(56)

**References Cited**

U.S. PATENT DOCUMENTS

|                  |         |                                           |
|------------------|---------|-------------------------------------------|
| 5,200,036 A      | 4/1993  | Noda                                      |
| 5,279,767 A      | 1/1994  | Phan et al.                               |
| 5,814,188 A      | 9/1998  | Vinson et al.                             |
| 6,416,624 B1     | 7/2002  | Nielsen et al.                            |
| 7,195,771 B1     | 3/2007  | Hsu et al.                                |
| 8,187,419 B2     | 5/2012  | Chan et al.                               |
| 2004/0074622 A1  | 4/2004  | Liu et al.                                |
| 2005/0238700 A1* | 10/2005 | Kleinwaechter .... A61K 8/0208<br>424/443 |
| 2005/0271710 A1  | 12/2005 | Argo et al.                               |
| 2006/0163524 A1  | 7/2006  | Lange et al.                              |
| 2006/0243405 A1* | 11/2006 | Zwick ..... D21H 21/22<br>162/135         |
| 2007/0044930 A1  | 3/2007  | Vinson et al.                             |
| 2007/0071797 A1  | 3/2007  | Hernandez-Munoa et al.                    |

(Continued)

FOREIGN PATENT DOCUMENTS

|    |             |         |
|----|-------------|---------|
| CN | 104099809 A | 10/2014 |
| EP | 0803012 B1  | 6/1999  |

(Continued)

OTHER PUBLICATIONS

Ghosh, A.K., Fundamentals of Paper Drying—Theory and Application from Industrial Perspective. Evaporation, Condensation and Heat transfer, Sep. 12, 2011, pp. 574-575.

Co-pending U.S. Appl. No. 16/084,281, filed Sep. 12, 2018, by Lee et al. for "Tissue Comprising a Softening Composition."

*Primary Examiner* — Jose A Fortuna

(74) *Attorney, Agent, or Firm* — Kimberly-Clark Worldwide, Inc.

(57) **ABSTRACT**

A soft through-air dried tissue having a soothing feel and method of making the same is disclosed which contains an aqueous softening composition comprising from about 10 to about 20 weight percent of a cationic softening compound, such as quaternary ammonium compounds and imidazolinium compounds; from about 10 to about 20 weight percent of a polyhydroxy compound having a molecular weight of at least about 1,000 g/mol, and optionally a silicone or glycerin. Examples of the cationic softening compound include tallow- and ester-substituted quaternary ammonium compounds having chloride or methyl sulfate as the anion, and examples of the polyhydroxy compound include polyethylene glycols (PEG) or polypropylene glycols (PPG) having a molecular weight of at least about 1,000 g/mol, such as PEG-1000 and PEG-8000.

(56)

**References Cited**

U.S. PATENT DOCUMENTS

2007/0196405 A1 8/2007 Wilker et al.  
2009/0188637 A1\* 7/2009 Chan ..... D21H 17/33  
162/112  
2009/0297781 A1\* 12/2009 Huss ..... B31F 1/07  
428/166  
2009/0314444 A1 12/2009 Sorns et al.  
2010/0155004 A1 6/2010 Soerens et al.  
2010/0236735 A1\* 9/2010 Goulet ..... D21H 17/34  
162/112  
2011/0217345 A1\* 9/2011 Huang ..... C08K 5/05  
424/401  
2014/0037701 A1\* 2/2014 Mellin ..... A61K 8/31  
424/401  
2014/0037896 A1\* 2/2014 Ho-Kleinwaechter .....  
B32B 29/005  
428/125  
2015/0159330 A1 6/2015 Weisman et al.  
2016/0244915 A1\* 8/2016 Mohammadi ..... D21H 19/10  
2017/0009402 A1\* 1/2017 Mohammadi ..... C11D 3/2093  
2018/0094388 A1\* 4/2018 Mohammadi ..... D21H 17/53  
2019/0002747 A1\* 1/2019 Salaam-Zayid ..... C09K 5/06  
2019/0031802 A1 1/2019 Gu et al.  
2019/0071822 A1\* 3/2019 Lee ..... D21H 27/00  
2019/0078262 A1\* 3/2019 Vogt ..... D21H 27/004

FOREIGN PATENT DOCUMENTS

EP 1408155 B1 12/2006  
JP 10226986 A2 8/1998  
WO WO9906634 A1 2/1999

\* cited by examiner

## LOTION TREATED THROUGH-AIR DRIED TISSUE

### BACKGROUND OF THE DISCLOSURE

Tissue products, and particularly bath and facial tissue products, are often used for wiping and cleaning of the body. When wiping frequently with such products certain users may experience irritation and inflammation. Often the irritation and inflammation is caused in-part by the tissue product having a relatively rough surface.

There have been numerous previous attempts to correct the problem of irritation and inflammation caused by wiping with tissue products. One common approach has been to provide a tissue product which is smoother, softer, or both smoother and softer than previous products. One means of producing such a product involves applying a chemical additive to the product's surface. For example, chemical debonders that interfere with the natural fiber-to-fiber bonding may be added to the tissue product. The reduction in fiber-to-fiber bonding may be used to produce a softer, less harsh, product. Exemplary chemical debonding agents include quaternary ammonium salts such as trimethylco-coammonium chloride, trimethyloleylammonium chloride, dimethyldi(hydrogenated-tallow)ammonium methyl sulfate and trimethylstearylammmonium chloride. Mono or diester variations of the before mentioned quaternary ammonium salts have also been taught for use in the manufacture of tissue products.

Others have attempted to produce a soft tissue product by applying lotions comprising one or more oils, such as mineral oil, waxes, such as paraffin, or plant extracts, such as chamomile and aloe vera, to the tissue product. This approach has been applied by, for example, by Krzysik, et al., U.S. Pat. No. 5,885,697 and Warner, et al., U.S. Pat. No. 5,525,345.

Despite these efforts the problem of irritation and inflammation resulting from use of tissue products persists. Accordingly, it is an objective of the present invention to provide a tissue paper product which causes less irritation and inflammation to a user's skin. It is a further objective of this invention to provide a treated tissue paper product having a softening composition disposed thereon, where the tissue products has improved surface properties, such as a reduced coefficient of friction. It is yet a further objective of the present invention to provide an aqueous softening composition that may be easily and effectively applied to a tissue product using a wide variety of methods.

These and other objectives are obtained using the present invention, as will become readily apparent from a reading of the following disclosure.

### SUMMARY OF THE DISCLOSURE

It has now been discovered that the softness (measured as coefficient of friction) of a tissue web, and more particularly a through-air dried tissue web and still more particularly an uncreped through-air dried tissue web, may be met or exceeded without excessive use of softening compositions, such as lotions. More specifically it has been discovered that an aqueous softening composition comprising a cationic softening compound (hereinafter often called a "cationic softener"), such as a quaternary ammonium, and a relatively high molecular weight of polyhydroxy compound, such as a polyethylene glycol having a molecular weight of at least about 1,000 g/mol, may be applied at relatively low add-on levels, such as less than about 12 percent, by weight of the

tissue web, and still reduce the tissue's coefficient of friction (COF). In addition to a reduced COF, and despite the relatively modest amount of softening composition added to the web, the resulting tissue product may also provide an improved moisturizing feeling.

For example, by treating a tissue web with an aqueous softening composition comprising a cationic softening compound and a polyhydroxy compound having a molecular weight of at least about 1,000 g/mol, a tissue web that is both sufficiently strong to withstand use, such as a tissue product having a geometric mean tensile (GMT) from about 700 to about 1,500 g/3" and more preferably from about 800 to about 1,000 g/3", and having a low coefficient of friction, such as a tissue having a COF less than about 300 g, and more preferably less than about 250 g and still more preferably less than about 200 g, may be produced. Moreover, these product properties may be achieved despite applying less than about 12 dry weight percent, by weight of the tissue product, and in certain embodiments less than about 10 dry weight percent, such as from about 0.5 to about 12 dry weight percent, by weight of the tissue product, of softening composition to the tissue web. This discovery provides the flexibility to produce a tissue product with satisfactory softness at a given tensile strength while reducing the add-on of softening composition.

Hence, in one embodiment, the present invention provides a through-air dried tissue product produced by dispersing a furnish to form a fiber slurry; forming a wet tissue web; partially dewatering the wet tissue web; through-air drying the partially dewatered web to yield a dried tissue web; and topically applying an aqueous softening composition to the dried tissue web, the aqueous softening composition comprising a cationic softening compound and a polyhydroxy compound having a molecular weight of at least about 1,000 g/mol at add on levels less than about 12 dry weight percent, by weight of the dried tissue web.

Tissue webs produced by the foregoing process may be subject to additional converting, such as calendering or embossing, and may be combined to form multi-ply tissue products. Thus, in other embodiments the present invention provides a tissue product comprising at least one tissue web having an aqueous softening composition comprising a cationic softening compound and a polyhydroxy compound having a molecular weight of at least about 1,000 g/mol disposed thereon, the tissue product having a basis weight greater than about 25 grams per square meter (gsm), a GMT greater than about 700 g/3" and a COF less than about 300 g such as from about 100 to about 300 g and more preferably from about 175 to about 225 g.

In other embodiments the present invention provides a through-air dried tissue product comprising at least one tissue web that has been topically treated with an aqueous softening composition comprising a cationic softening compound and a polyhydroxy compound having a molecular weight of at least about 1,000 g/mol wherein the add on level of the aqueous softening composition is less than about 12 dry weight percent, by weight of the tissue web, the tissue product having a GMT greater than about 700 g/3" and a COF from about 175 to about 225 g.

In still other embodiments the invention provides a tissue product comprising at least one tissue web having a first and an opposed second surface, an aqueous softening composition disposed on the first or the second surface, the aqueous softening composition comprising (i) water; (ii) a polyhydroxy compound selected from the group consisting of glycerol, polyethylene glycols and polypropylene glycols, the polyhydroxy compound having a molecular weight at

least about 1,000 g/mol and (iii) a quaternary ammonium compound or an imidazoline compound.

In yet other embodiments the present invention provides a tissue product comprising two or more lotion treated tissue plies, each lotion treated tissue ply prepared by adding less than about 10 dry weight percent, by weight of the tissue web, of an aqueous softening composition consisting essentially of water, a quaternary ammonium compound, polyethylene glycol having a molecular weight from about 1,000 to about 10,000 g/mol and optionally a silicone or glycerin, or mixtures thereof, the tissue product having a GMT greater than about 700 g/3" and a COF from about 175 to about 225 g.

In other embodiments the present invention provides an aqueous softening composition useful in the manufacture of tissue webs and products, the composition comprising a cationic softening compound and a polyhydroxy compound having a molecular weight of at least about 1,000 g/mol and optionally a silicone or glycerin, wherein the mass ratio of water to the polyhydroxy compound is from about 1:0.5 to about 1:10. In a particularly preferred embodiment the water comprises from about 40 to about 80 weight percent, by weight of the softening composition.

In other embodiments the present invention provides an aqueous softening composition useful in the manufacture of tissue webs and products, the composition comprising (a) from about 0.1 to about 5.0 weight percent of silicone; (b) from about 10 to about 20 weight percent of a cationic softening compound; (c) from about 10 to about 20 weight percent of a polyhydroxy compound having a molecular weight of at least about 1,000 g/mol; (d) from about 10 to about 30 weight percent glycerin and (e) from about 25 to 70 weight percent water. In a particularly preferred embodiment the foregoing composition components (a)-(d) comprise from 30 to about 75 weight percent of the composition. Generally the foregoing aqueous softening composition is topically applied to a tissue web at add-on levels from about 0.5 to 5.0 dry weight percent, based upon the dry weight of the tissue, for improving softness and moisturizing feeling of the tissue web.

#### DEFINITIONS

As used herein the term "add-on" refers to the amount of softening composition, on a dry weight basis, added to the tissue web or product. Add-on may be calculated by determining the dry weight of the softening composition added to the web or product and dividing by the bone dry basis weight of the web or product. For example, if 5.0 grams of softening composition comprising 40 percent solids is added to a tissue web having a bone dry basis weight of 40 gsm, the add-on is 5.0 percent.

As used herein the term "emulsion" refers to a heterogeneous mixture of generally an insoluble liquid comprising an aqueous phase and an organic phase. Generally, for aqueous softening compositions of the present invention, the aqueous phase comprises water, which is used to emulsify the cationic softening compound and the polyhydroxy compound.

As used herein, the term "basis weight" generally refers to the bone dry weight per unit area of a tissue and is generally expressed as grams per square meter (gsm). Basis weight is measured using TAPPI test method T-220. Normally, the basis weight of a tissue product of the present invention is less than about 80 grams per square meter (gsm), in some embodiments less than about 60 gsm, and in some embodiments from about 10 to about 60 gsm and more preferably from about 20 to about 50 gsm.

As used herein, the term "caliper" is the representative thickness of a single sheet (caliper of tissue products comprising two or more plies is the thickness of a single sheet of tissue product comprising all plies) measured in accordance with TAPPI test method T402 using a ProGage 500 Thickness Tester (Thwing-Albert Instrument Company, West Berlin, N.J.). The micrometer has an anvil diameter of 2.22 inches (56.4 mm) and an anvil pressure of 132 grams per square inch (per 6.45 square centimeters) (2.0 kPa).

As used herein, the term "Coefficient of Friction" (COF) refers to the root mean square of the machine direction (MD) and cross-machine direction (CD) COF measured as described in the Test Methods section below. While the COF may vary depending on the tissue web to be treated, the composition of the softener and the add-on amount, tissue products and webs produced as described herein generally have a COF less than about 300 g, more preferably less than about 250 g and still more preferably less than about 200 g. In certain embodiments inventive tissue products may have a COF from about 100 to about 300 g, more preferably from about 150 to about 250 g and still more preferably from about 175 to about 225 g.

As used herein, the term "sheet bulk" refers to the quotient of the sheet caliper (generally having units of  $\mu\text{m}$ ) divided by the bone dry basis weight (generally having units of gsm). The resulting sheet bulk is expressed in cubic centimeters per gram (cc/g). While the sheet bulk of the products prepared according to the present invention may vary depending on the method of manufacture, the tissue products generally have a sheet bulk greater than about 10.0 cc/g such as from about 10.0 to about 20.0 cc/g and more preferably from about 12.0 to about 15.0 cc/g.

The term "ply" refers to a discrete product element. Individual plies may be arranged in juxtaposition to each other. The term may refer to a plurality of web-like components such as in a multi-ply facial tissue, bath tissue, paper towel, wipe, or napkin.

As used herein, the term "slope" refers to slope of the line resulting from plotting tensile versus stretch and is an output of the MTS TestWorks™ in the course of determining the tensile strength as described in the Test Methods section herein. Slope is reported in the units of mass per unit of sample width and is measured as the slope of the least-squares line fitted to the load-corrected strain points falling between a specimen-generated force of 70 to 157 grams (0.687 to 1.540 N) divided by the specimen width. Slopes are generally reported herein as having units of grams force (gf) or kilograms force (kgf).

As used herein, the term "geometric mean slope" (GM Slope) generally refers to the square root of the product of machine direction slope and cross-machine direction slope. GM Slope generally is expressed in units of kilograms (kg).

As used herein, the term "geometric mean tensile" (GMT) refers to the square root of the product of the machine direction tensile strength and the cross-machine direction tensile strength of the web.

While the GMT may vary, tissue products prepared according to the present disclosure generally have a GMT greater than about 500 g/3", such as from about 500 to about 1,500 g/3" and more preferably from about 750 to about 1,000 g/3".

As used herein, the term "Stiffness Index" refers to the quotient of the geometric mean tensile slope, defined as the square root of the product of the MD and CD slopes (typically having units of kgf), divided by the geometric mean tensile strength (typically having units of gf).

Stiffness Index =

$$\frac{\sqrt{MD \text{ Tensile Slope (kgf)} \times CD \text{ Tensile Slope (kgf)}}}{GMT \text{ (gf)}} \times 1,000$$

While the Stiffness Index may vary tissue products prepared according to the present disclosure generally have a Stiffness Index less than about 20 and more preferably less than about 15, such as from about 10 to about 20 and more preferably from about 10 to about 15.

As used herein, a "tissue product" generally refers to various paper products, such as facial tissue, bath tissue, paper towels, napkins, and the like. Tissue products may comprise one, two, three or more plies. The tissue product may be a web of tissue spirally wound onto a core or may comprise individual folded sheets that may be stacked together.

The term "dry tissue web" as used herein includes both webs which are dried to a moisture content less than the equilibrium moisture content thereof and webs which are at a moisture content in equilibrium with atmospheric moisture.

All percentages, ratios and proportions herein are by weight, unless otherwise specified.

#### DETAILED DESCRIPTION OF THE DISCLOSURE

It was previously believed that softening compositions, such as silicones, glycerin, or waxes, needed to be added at high levels, with greater reductions in tensile strength, to achieve soft tissue products (often measured as low levels of friction). It has now been surprisingly discovered that the add-on of softening composition may be reduced significantly by applying an aqueous softening composition comprising a cationic softening compound and a relatively high molecular weight of polyhydroxy compound to the tissue web.

Thus, the present invention provides a tissue web having a softness that meets or exceeds satisfactory levels without the excess use of softening compositions, such as lotions. The satisfactory level of softness, which may be measured as coefficient of friction (COF), is generally less than about 300 g, more preferably less than about 250 g and still more preferably less than about 225 g. In certain embodiments inventive tissue products may have a COF from about 100 to about 300 g, more preferably from about 150 to about 250 g and still more preferably from about 175 to about 225 g.

The satisfactory level of softness on at least one surface of the tissue web may be achieved by applying relatively low levels of the aqueous softening composition to the surface of the tissue web, such as less than about 12 dry weight percent, by weight of the dry tissue web, and more preferably less than about 10 percent and still more preferably less than about 6.0 percent and still more preferably less than about 4.0 percent. In certain embodiments the total softening composition add-on may range from about 0.5 to about 12 dry weight percent, by weight of the dry tissue web, such as from about 0.5 to about 10.0 and more preferably from about 0.5 to about 5.0. The foregoing add-on levels not only achieve a relatively low coefficient of friction, such as less than about 300 g, but also result in tissue products with a surprisingly high degree of strength, such as a GMT greater than about 500 g/3", such as from about 500 to about 1,500

g/3", more preferably from about 700 to about 1,100 g/3" and more preferably from about 800 to about 1,000 g/3".

Tissue webs and products may be manufactured by applying an aqueous softening composition comprising a cationic softening compound and a relatively high molecular weight of polyhydroxy compound to at least one surface of the web. Suitable cationic softening compounds include both quaternary ammonium compounds including, for example, amidoamine quaternary ammonium compounds, diamidoamine 10 quaternary ammonium compounds, ester quaternary ammonium compounds, alkoxy alkyl quaternary ammonium compounds, benzyl quaternary ammonium compounds, alkyl quaternary ammonium compounds, and imidazolinium compounds.

15 For example, in one embodiment, the softening composition comprises an alkyl quaternary ammonium compound having the general formula:



20 where R1' is a C<sub>1-6</sub> alkyl group, R1'' is a C<sub>14-22</sub> alkyl group, b is an integer from 1 to 3 and X- is any suitable counterion such as, acetate, chloride, bromide, methylsulfate, formate, sulfate, nitrate.

In certain preferred embodiments the quaternary ammonium compound is a natural or synthetic tallow where R1'' is a C<sub>16-18</sub> alkyl and more preferably where R1'' is straight-chain C<sub>18</sub> alkyl. In those instances where the quaternary ammonium compound is derived from natural sources, several different types of vegetable oils may be used, such 25 as olive, canola, safflower, or sunflower oil. Suitable quaternary ammonium compounds include, for example, dialkyldimethylammonium salts (e.g., ditallowdimethylammonium chloride, ditallowdimethylammonium methyl sulfate, di(hydrogenated tallow)dimethyl ammonium chloride, etc.) and trialkylmethylammonium salts (e.g., tritallowmethylammonium chloride, tritallowmethylammonium methyl sulfate, tri(hydrogenated tallow)methyl ammonium chloride, etc.), in which R1' are methyl groups and R1'' are 30 tallow groups of varying levels of saturation. X- can be any compatible anion such as, acetate, chloride, bromide, methylsulfate, and formate. In a particularly preferred embodiment X- is chloride or methyl sulfate.

In other embodiments the quaternary ammonium compound comprises mono-, di-, or tri-ester quaternary ammonium compounds; di-esterified quaternary ammonium compounds having the general formula:



where Y is —O—(O)C—, or —C(O)—O—, or —NH—C 50 (O)—, or —C(O)—NH—; b is 1 to 3; n is 0 to 4; R1' is a C<sub>1-6</sub> alkyl group, hydroxyalkyl group, hydrocarbyl or substituted hydrocarbyl group, alkoxyalated group, benzyl group, or mixtures thereof; R1'' is a C<sub>13-21</sub> alkyl group, hydroxyalkyl group, hydrocarbyl or substituted hydrocarbyl 55 group, alkoxyalated group, benzyl group, or mixtures thereof; and X is any softener-compatible anion. In a particularly preferred embodiment Y=—O—(O)C—, or —C(O)—O—; b=2; and n=2. In other embodiments R1' is a C<sub>1-3</sub>, alkyl group, with methyl being most preferred. In still other 60 embodiments R1'' is C<sub>13-18</sub> alkyl and/or alkenyl, more preferably R1'' is straight chain C<sub>15-18</sub> alkyl and/or alkenyl. Optionally, the R1'' substituent can be derived from vegetable oil sources such as olive, canola, safflower, or sunflower oil. As noted previously, X- can be any compatible anion such as, acetate, chloride, bromide, methylsulfate, 65 formate, and nitrate. Preferably X- is chloride or methyl sulfate.

In one particularly preferred embodiment the cationic softener comprises ester quaternary ammonium compounds such as those marked under the tradename SUNQAT-CEQ90 (Sunjin Chemical Co. Ltd., Ansan, South Korea).

In other embodiments the softening composition may comprise imidazolinium compounds having the general formula:



wherein R<sup>1</sup> and R<sup>2</sup> are each independently a C<sub>12-20</sub> hydrocarbyl group. Therefore, R<sup>1</sup> and R<sup>2</sup> can be the same or different. Although not illustrated the imidazolinium compound is typically provided with a compatible anion.

Preferred imidazolinium compounds are those imidazoline derivatives wherein R<sup>1</sup> and R<sup>2</sup> are independently C<sub>12-20</sub> alkyl and alkenyl, and more preferably C<sub>14-20</sub> alkyl. Suitable examples of such imidazoline derivatives include stearyl amido ethyl-2-stearyl imidazoline, stearyl amido ethyl-2-palmityl imidazoline, stearyl amido ethyl-2-myristyl imidazoline, palmityl amido ethyl-2-palmityl imidazoline, palmityl amido ethyl-2-myristyl imidazoline, stearyl amido ethyl-2-tallow imidazoline, myristyl amido ethyl-2-tallow imidazoline, palmityl amido ethyl-2-tallow imidazoline, coconutamido ethyl-2-coconut imidazoline, tallow amido ethyl-2-tallow imidazoline and mixtures of such imidazoline derivatives. More preferred are those imidazoline derivatives wherein R<sup>1</sup> and R<sup>2</sup> are independently C<sub>16-20</sub> alkyl (e.g. wherein R<sup>1</sup> and R<sup>2</sup> are palmityl, stearyl and arachidyl). Most preferred are those imidazoline compounds wherein R<sup>1</sup> and R<sup>2</sup> are independently C<sub>16-18</sub> alkyl, i.e., wherein R<sup>1</sup> and R<sup>2</sup> are each derived from tallow.

Particularly preferred imidazoline-derivatives include cationic oleyl imidazoline materials such as methyl-1-oleylamidoethyl-2-oleylimidazolinium methylsulfate commercially available as Mackernium CD-183 (McIntyre Ltd., University Park, Ill.) and Prosoft TQ-1003 (Solenis LLC, Wilmington, Del.) of which cationic portion having the formula:



The cationic softening compound may be incorporated in the softening composition of the present invention in varying amounts. For example, in one embodiment the cationic softening compound may comprise from about 5.0 to about 30 weight percent, by weight of the softening composition, more preferably from about 8.0 to about 20 weight percent and still more preferably from about 10 to about 15 weight percent.

In addition to a cationic softening compound, the softening composition contains a polyhydroxy compound and

more preferably a relatively high molecule weight polyhydroxy compound, such as a polyhydroxy compound having a molecular weight of at least about 1,000 g/mol. A particularly preferred polyhydroxy compound has a molecular weight of greater than about 4,000 g/mol. As such the molecule weight of polyhydroxy compound may range from about 1,000 to about 12,000 g/mol and more preferably from about 1,500 to about 10,000 g/mol and still more preferably from about 6,000 to about 8,000 g/mol.

- 10 Examples of polyhydroxy compounds useful in the present invention include, but are not limited to, polyethylene glycols and polypropylene glycols having a molecular weight of at least about 1,000 g/mol and more preferably greater than about 2,000 g/mol and still more preferably greater than about 4,000 g/mol and more preferably greater than about 6,000 g/mol, such as from about 1,000 to about 12,000 g/mol, and more preferably from about 4,000 to about 10,000 g/mol and still more preferably from about 6,000 to about 8,000 g/mol. In a particularly preferred embodiment, the softening composition comprises a polyethylene glycol having a molecular weight of from about 1,000 to about 10,000 g/mol and more preferably from about 6,000 to about 8,000 g/mol.

In certain embodiments the softening composition may comprise two or more different polyhydroxy compounds, such as polyethylene glycol of different molecular weights. Thus, in one particularly preferred embodiment the softening composition comprises a first polyethylene glycol having a molecular weight from about 1,000 to about 6,000 g/mol and a second polyethylene glycol having a molecular weight from about 8,000 to about 10,000 g/mol.

The polyhydroxy compound may be incorporated in the softening composition of the present invention in varying amounts. In one embodiment the polyhydroxy compound comprises from about 5.0 to about 30 weight percent, by weight of the softening composition, more preferably from about 8.0 to about 20 weight percent and still more preferably from about 10 to about 15 weight percent.

The relative ratio of the cationic softener to the polyhydroxy compound may be varied to achieve the desired tissue product properties or to accommodate different methods of application. For example, in certain embodiments, the weight ratio of the cationic softener to the polyhydroxy compound ranges from about 1:0.1 to about 0.1:1, and more preferably from about 1:0.3 to about 0.3:1 and still more preferably from about 1:0.7 to about 0.7:1, although this ratio will vary depending upon the molecular weight of the particular cationic softener and polyhydroxy compound used.

- 50 The foregoing softening composition is generally applied to one or two outermost surfaces of a dry tissue web and more preferably a creped tissue web. As such the softening composition is generally applied as an aqueous solution comprising a cationic softening compound and polyhydroxy compound. The aqueous softening solution is generally prepared as a water-based emulsion and then applied to the dry tissue web. It is believed in this manner that tactile softness of the tissue sheet and resulting tissue products may be improved due to presence of the softening composition 55 on the surface of the tissue product. Thus, the aqueous softening composition generally comprises from about 25 to about 75 weight percent, by weight of the composition, water and more preferably from about 30 to about 60 percent and still more preferably from about 40 to about 50 percent.
- 60 In other embodiments the amount of water in the aqueous softening composition may be varied depending upon the amount of the polyhydroxy compound. For example the

mass ratio of water to the polyhydroxy compound may be about 1:0.1 to about 1:10 and more preferably from about 1:0.2 to about 1:5 and still more preferably from about 1:0.5 to about 1:2. In a particularly preferred embodiment the water comprises from about 40 to about 80 weight percent, by weight of the softening composition, and the polyhydroxy compound comprises from about 10 to about 15 weight percent.

To further enhance softening of the tissue sheet and resulting tissue products the softening composition may also include a silicone, also referred to herein as a polysiloxane or as a siloxane. A large variety of silicones are available that are capable of enhancing the tactile properties of the finished tissue sheet. Any silicone capable of enhancing the tactile softness of the tissue sheet is suitable for incorporation in this manner so long as solutions or emulsions of the cationic softener and silicone are compatible, that is when mixed they do not form gels, precipitates or other physical defects that would preclude application to the tissue sheet.

Examples of suitable silicones include but are not limited to linear polydiallyl polysiloxanes such as the DC-200 fluid series available from Dow Corning, Inc., Midland, Mich., as well as the organo-reactive polydimethyl siloxanes such as the preferred amino functional polydimethyl siloxanes. Examples of suitable silicones include those described in U.S. Pat. Nos. 6,054,020 and 6,432,270, the disclosures of which are incorporated herein by reference in a manner consistent with the instant disclosure. Suitable silicones generally have the formula:



wherein:

X is hydrogen, hydroxy, amino,  $C_{1-8}$  straight chain, branched, cyclic, unsubstituted or hydrophilically substituted alkyl or alkoxy radical;

$m=20-100,000$ ;

$p=1-5000$ ;

$q=0-5000$ ;

$R_1=a C_{1-6}$ , straight chain, branched or cyclic alkyl radical;

$R_2=a C_{1-10}$  straight chain or branched, substituted or unsubstituted alkylene diradical;



wherein:

$R_5$  is an unsubstituted or a hydrophilically substituted  $C_{1-10}$  alkylene diradical;

$r=1-10,000$ ;

$s=0-10,000$ ; and

Z=hydrogen,  $C_{1-24}$  alkyl group, or a G-group, where G is selected from the following:  $— R_6 \text{COOR}_7$ ;  $— \text{CONR}_8 \text{R}_9$ ;  $— \text{SO}_3 \text{R}_8$ ; and  $\text{PO R}_8 \text{R}_9$ , where  $R_6$  is a substituted or unsubstituted  $C_{1-6}$  alkylene diradical;  $R_7$ ,  $R_8$ , and  $R_9$  are independently a hydrogen radical or a substituted or unsubstituted  $C_{1-8}$  alkyl radical; and



5

wherein:

$R_{10}$ ,  $R_{11}$ , and  $R_{12}$  are independently an unsubstituted or a hydrophilically substituted  $C_{1-8}$  alkylene diradical;

$t=0-10,000$ ;

$u=0-10,000$ ;

$w=0-10,000$ ; and

$R_{13}$ ,  $R_{14}$  and  $R_{15}$  are independently a hydrogen radical, an unsubstituted or a hydroxyl, carboxyl or other functionally substituted  $C_{1-10}$  straight chain, branched, or cyclic alkyl radical.

When incorporated in the softening composition, silicone may be added at varying amounts. In one embodiment the softening composition comprises at least about 0.1 weight percent, by weight of the softening composition, silicone, such as from about 0.1 to about 6.0 dry weight percent, and more preferably from about 0.1 to about 5.0 weight percent and still more preferably from about 0.5 to about 3.0 weight percent.

While silicone may be incorporated in the softening composition of the present invention, its presence is not necessary. Surprisingly, in certain embodiments, a soft tissue product, such as a tissue product having a COF less than about 300 and more preferably less than about 250 and still more preferably less than about 225 g, may be prepared with the addition of little or no silicone. For example, the foregoing properties may be achieved by applying an aqueous softening composition comprising less than about 0.5 weight percent silicone, such as from about 0 to about 0.5 weight percent silicone.

In still other embodiments, the softening composition may optionally include glycerin. When incorporated in the softening composition, the amount of glycerin in the softening composition can be from about 5.0 to about 40 weight percent, more particularly from about 10 to about 30 weight percent, and still more particularly from about 15 to about 20 weight percent.

Thus, in certain embodiments the softening composition of the present invention may consist essentially of water, a cationic softening compound, such as a quaternary ammonium compound, a polyhydroxy compound having a molecular weight of at least about 1,000 g/mol and optionally a silicone or glycerin, or mixtures thereof. In other embodiments the softening composition may consist essentially of water, a quaternary ammonium compound, a polyhydroxy compound having a molecular weight of at least about 1,000 g/mol, a silicone and glycerin.

Other chemicals commonly used in papermaking can be added to the softening composition described herein, or to the papermaking furnish so long as they do not significantly and adversely affect important tissue product properties, such as strength or absorbency of the tissue product, or negatively affect the softening provided by the softening compositions of the present invention. For example, dry strength additives such as starch or carboxymethyl cellulose may be added to the furnish to improve the tensile strength of the tissue products. In other embodiments wet strength resins, such as polyamide-epichlorohydrin resins may be added to the furnish to improve the tensile strength of the tissue product when wet. In still other embodiments a

## 11

temporary wet strength agent may be added to the furnish, such as modified starch and more particularly cationic starches.

Other additives may include humectants and skin protectants. Suitable humectants include lactic acid and its salts, sugars, ethoxylated glycerin, ethoxylated lanolin, corn syrup, hydrolyzed starch hydrolysate, urea, and sorbitol. Suitable skin protectants include allantoin, kaolin, zinc oxide, aloe vera, vitamin E, petrolatum and lanolin. Again, the foregoing additives are generally complementary to the softening compositions of the present invention and generally do not significantly and adversely affect important tissue product properties, such as strength or absorbency of the tissue product, or negatively affect the softening provided by the softening compositions of the present invention.

The softening composition of the present invention may be added to the tissue web at any point after the web has been formed and at least partially dewatered. In a particularly preferred embodiment the softening composition is applied to the web after it has been dried to final dryness, such as a moisture content less than about 6.0 percent (by weight of the tissue web) and more preferably less than about 5.0 percent. For example, the softening composition may be applied after the drying section of the tissue machine where the tissue sheet has a consistency of from about 90 to about 100 percent. The softening composition may also be applied via a secondary post treatment process where the tissue sheet has a consistency of from about 90 to about 100 percent.

The method by which the softening composition is applied to the tissue sheet may be accomplished by any method known in the art. For example, in one embodiment the composition may be applied by contact printing methods such as gravure, offset gravure, flexographic printing and the like. The contact printing methods often enable topical application of the composition to the tissue sheet. In other embodiments the softening composition may be applied to the tissue web by non-contact printing methods such as ink jet printing, digital printing of any kind, and the like.

In still other embodiments the softening composition may be sprayed onto the tissue sheet. For example, spray nozzles may be mounted over a moving tissue sheet to apply a desired dose of a solution to the tissue sheet. Nebulizers may also be used to apply a light mist to a surface of a tissue sheet. In other embodiments the softening composition may be applied to a moving belt or fabric by spray or other means and the belt or fabric may in-turn contact the tissue sheet to apply the softening composition to the tissue web. In still other embodiments the softening composition may be applied by coating onto the tissue sheet by slot coating, blade coating, air knife coating, short dwell coating, cast coating, and the like.

Preferred methods of application include gravure printing, flexographic printing, spraying and topical application using a WEKO fluid application system (commercially available from Weitmann & Konrad GmbH & Co., Leinfelden-Echterdingen, Germany). A particularly preferred method of application is rotogravure printing such as described in U.S. Pat. No. 5,665,426, the contents of which are incorporated herein by reference in a manner consistent with the present disclosure.

In one embodiment the softening composition may be applied by an indirect application process where the softening composition is applied to the web via a transfer/applicator roll. For example, the web to be treated may be threaded from an unwind roll through a nip between the transfer/applicator roll and a backing roll. The softening

## 12

composition is added to a second nip created between a Mayer rod and the transfer/applicator roll. Mayer rods are well known in the art and are provided in a number of different configurations that allow different volumes of fluid to be put onto the transfer/applicator roll. The softening composition applied to the transfer/applicator roll by the Mayer rod is subsequently disposed on the web.

The softening composition may be applied to only a single surface of the tissue web or may be applied to both the upper and opposed lower surfaces of the web. The add-on amount of the softening composition on each surface of the tissue web can be from about 0.25 to about 6.0 dry weight percent based on the weight of the tissue, more specifically from about 1.0 to about 5.0 dry weight percent, and still more specifically from about 1.0 to about 3.5 dry weight percent.

Further, it is generally desirable after formation and drying of the web to prevent significant rewetting of the tissue sheet or to negatively affect the web's tensile strength by topically applying excessive amounts of aqueous solution. Thus, in a preferred embodiment, the add-on amount of softening composition on one surface is less than about 6.0 dry weight percent and the addition of the softening composition results in a geometric mean tensile strength decrease of less than about 30 percent, as measured in the treated tissue sheet compared to the untreated tissue sheet. While having minimal negative effect on tensile strength the foregoing add-ons may reduce the coefficient of friction of an untreated tissue web by more than 20 percent, and in some instances by more than 25 percent, such as from about 20 to about 35 percent.

The reduction in COF may also be accompanied by improvements in other tissue product properties, such as the Stiffness Index. As such, in certain embodiments, tissue products prepared according to the present invention may have a GMT from about 700 to about 1,500 g/3" and more preferably from about 750 to about 1,000 g/3", a COF less than about 300 g and more preferably less than about 250 g, and still more preferably less than about 225 g and a Stiffness Index less than about 10.0, such as from about 5.00 to about 10.0 and more preferably from about 5.00 to about 8.00. The foregoing tissue products may be prepared despite adding less than about 10 dry weight percent, and in some instances less than about 5.0 dry weight percent, of softening composition.

In addition to providing surprisingly low coefficients of friction at a given add-on level, the instant softening compositions provide the additional benefit that they may be prepared as water-based emulsions that do not require further heating prior to use. Thus, in one embodiment, the softening composition is prepared and applied to the tissue as an emulsion comprising at least about 50 weight percent water (as a percent of the total weight of the emulsion). In other embodiments softening composition emulsions of the present invention may comprise from about 50 to about 90 weight percent of water, preferably 55 to 80 weight percent, and more preferably 60 to 75 weight percent.

The emulsion generally is not heated prior to application to the web and as such is generally applied at a temperature less than about 30° C., such as from about 15 to about 30° C. and more preferably from about 20 to about 25° C.

While the emulsion is preferably not heated prior to application, preparation of the emulsion may require heating of one or more of the components. For example, the emulsion may be prepared by heating the polyhydroxy compound to a temperature greater than about 50° C., such as from about 50 to about 70° C., and then adding the cationic

softener and mixing, followed by the addition of water and further mixing to form the emulsion. Upon mixing the emulsion generally has a viscosity from about 50 to about 1,000 cPs, such as from about 100 to about 800 cPs.

When applied to the tissue web, the softening composition can cover the entire surface area of the web or a portion of the web. For example, the composition can be applied so as to cover from about 20 to about 80 percent of the surface area of the web, and particularly from about 30 to about 60 percent of the surface area of the web. In certain embodiments, depending on the composition of the softening composition, leaving untreated areas on the web, the web remains easily wettable, which can be a concern when applying hydrophobic additives.

Without being bound by any particular theory, it is believed that premixing the cationic softening compound and the polyhydroxy compound prior to application to the tissue web enhances the retention of the polyhydroxy compound on the surface of the web and enhances surface softness. Thus, in certain embodiments, a high percentage of the polyhydroxy compound is retained on the surface of the web, such as at least about 40 percent and more preferably at least about 50 percent and still more preferably at least about 60 percent, such as from about 40 to about 95 percent. In a particularly preferred embodiment from about 70 to about 95 percent of the polyhydroxy compound is retained on the surface of the web.

Not only is a relatively high percentage of the polyhydroxy compound initially retained on the surface of the web, a significant amount of the polyhydroxy compound may remain on the surface well after formation of the resulting tissue product. While not wishing to be bound by theory, it is believed that the addition of both a cationic softening compound and a polyhydroxy compound and particularly a relatively high molecular weight, e.g., at least about 1,000 g/mol, polyhydroxy compound results in increased retention on the fiber surface and less z-directional migration. These relatively high molecular weights of polyhydroxy compound have relatively low glass transition temperatures, such as from about -20 to about -5 °C., and are good film forming agents, hence sheet stiffness and therefore tissue sheet softness is not negatively impacted by their presence. As such, tissue webs and products having the foregoing softening composition applied to at least one surface generally have equal or greater softness at higher tensile strength and lower add-on levels compared to other lotion treated tissue webs and products.

Thus, in one embodiment, the present invention provides a multi-ply tissue product comprising first and second outer plies and a third middle ply disposed between the first and second outer plies where the first and second outer plies comprise a tissue web comprising the softening composition of the present invention disposed on at least one surface, and the third middle ply is manufactured without the addition of softening composition. Despite the middle ply being manufactured without the addition of softening composition certain components of the softening composition applied to the outer plies may migrate through the outer plies to the middle ply. According, in certain embodiments from about 5.0 to about 20 weight percent of the total cationic softener found in the tissue product may be found in the middle layer and more preferably from about 5.0 to about 15 weight percent. Conversely, the middle layer is preferably substantially free from high molecular weights of polyhydroxy.

The softening composition of the present invention is useful in the manufacture of a wide variety of different tissue products. For most applications, however, the present invention

is directed to applying the softening composition to tissue products, particularly wiping products. Such products include, for example, facial tissues and bath tissues that have a basis weight of less than about 100 gsm, and particularly from about 20 to about 60 gsm, and more particularly from about 25 to about 45 gsm. The tissue web can be made exclusively of pulp fibers or, alternatively, can contain pulp fibers mixed with other fibers.

Besides bath and facial tissue products, however, the softening composition of the present invention can also be applied to paper towels and industrial wipers. Such products can have a basis weight of up to about 200 gsm and particularly up to about 150 gsm. Such products can be made from pulp fibers alone or in combination with other fibers, such as synthetic fibers. The pulp fibers can be softwood fibers, hardwood fibers, thermomechanical pulp, and the like.

The paper web treated in accordance with the present invention can also be formed by a variety of through-air drying processes known in the art. For example, the paper web treated in accordance with the present invention can be through-air dried, creped through-air dried, uncreped through-air dried, and the like. Examples of paper webs that can be used in the present invention include those disclosed in U.S. Pat. Nos. 5,048,589, 5,399,412 and 5,129,988, all of which are incorporated herein in a manner consistent with the present invention.

In one particular embodiment of the present application, the paper web treated in the process of the present invention is an uncreped through-air dried web. Uncreped through-air dried webs are generally formed in a wet paper making process in which a slurry of fibers is deposited onto a forming fabric. To dry the formed web, the web is fed through a through-air dryer while the web is being supported by a dryer fabric. Once formed, the web can have a fabric side that is generally softer to the touch than the opposite side of the web. In one embodiment of the present invention, a composition is applied opposite the fabric side and then transferred to the fabric side when wound into a roll. When applying, for instance, softeners to paper webs, less composition is generally needed on the fabric side.

## TEST METHODS

### 45 Basis Weight

The basis weight was measured as bone dry basis weight. Basis weight of the tissue sheet specimens may be determined using the TAPPI T410 procedure or a modified equivalent such as: Tissue samples are conditioned at 23±1° C. and 50±2 percent relative humidity for a minimum of 4 hours. After conditioning, a stack of 16 3-inch by 3-inch samples are cut using a die press and associated die. This represents a tissue sheet sample area of 144 in<sup>2</sup> or 929 cm<sup>2</sup>. Examples of suitable die presses are TMI DGD die press manufactured by Testing Machines, Inc., Islandia, N.Y., or a Swing Beam testing machine manufactured by USM Corporation, Wilmington, Mass. Die size tolerances are ±0.008 inches in both directions. The specimen stack is then weighed to the nearest 0.001 gram using an analytical balance. The basis weight in grams per square meter (gsm) is calculated using the following equation: Basis weight=stack weight in grams/0.0929.

### Tensile

Samples for tensile strength testing are prepared by cutting a 3 inches (76.2 mm) by 5 inches (127 mm) long strip in either the machine direction (MD) or cross-machine direction (CD) orientation using a JDC Precision Sample

Cutter (Thwing-Albert Instrument Company, Philadelphia, Pa., Model No. JDC 3-10, Ser. No. 37333). The instrument used for measuring tensile strengths is an MTS Systems Sintech 11S, Serial No. 6233. The data acquisition software is MTS TestWorks™ for Windows Ver. 4 (MTS Systems Corp., Research Triangle Park, N.C.). The load cell is selected from either a 50 Newton or 100 Newton maximum, depending on the strength of the sample being tested, such that the majority of peak load values fall between 10 and 90 percent of the load cell's full scale value. The gauge length between jaws is  $4\pm0.04$  inches. The jaws are operated using pneumatic-action and are rubber coated. The minimum grip face width is 3 inches (76.2 mm), and the approximate height of a jaw is 0.5 inches (12.7 mm). The crosshead speed is  $10\pm0.4$  inches/min (254±1 mm/min), and the break sensitivity is set at 65 percent. The sample is placed in the jaws of the instrument, centered both vertically and horizontally. The test is then started and ends when the specimen breaks. The peak load is recorded as either the "MD tensile strength" or the "CD tensile strength" of the specimen depending on the sample being tested. At least six (6) representative specimens are tested for each product, taken "as is," and the arithmetic average of all individual specimen tests is either the MD or CD tensile strength for the product.

#### Coefficient of Friction

Coefficient of friction ("COF") was determined using an MTS Systems Sintech 11S, Serial No. 6233. The data acquisition software is MTS TestWorks™ for Windows Ver. 4 (MTS Systems Corp., Research Triangle Park, N.C.). Samples are prepared by cutting a 3 inches (76.2 mm) by 5 inches (127 mm) long strip in the machine direction (MD) using a JDC Precision Sample Cutter (Thwing-Albert Instrument Company, Philadelphia, Pa., Model No. JDC 3-10, Ser. No. 37333). Samples were conditioned at  $23\pm1^\circ\text{C}$ . and  $50\pm2$  percent relative humidity for a minimum of 4 hours prior to testing.

The MD coefficient of friction was analyzed by placing three cut sheets of the basesheet material or finished tissue, treated side up, on the testing bed. The sample was secured to the testing bed by a clasp or double-sided tape. A single sheet of corresponding basesheet material or finished tissue specimen is attached to the COF testing sled with the treated side in facing arrangement with the treated side of the sample on the test bed. The samples were aligned with one another in the MD. Once the samples are affixed and arranged the test protocol is initiated to advance the sled. All COF units are in grams. Specific test parameters were as follows—Sled size: 1.5"×1.5"; Sled weight:  $200\pm5$  g; Sled Speed: 45 inches/min. Sliding Distance: 4"; Area of Measurement: 2" to 3.5"; Data acquisition rate: 20 Hz. The static coefficient of friction, also referred to as the peak load force, output by the data acquisition software is reported as the COF and typically has units of grams force (gf) or simply grams (g).

#### EXAMPLES

Base sheets were made using a through-air dried paper-making process commonly referred to as "uncreped through-air dried" ("UCTAD") and generally described in U.S. Pat. No. 5,607,551, the contents of which are incorporated herein in a manner consistent with the present invention. Base sheets with a target bone dry basis weight of about 46 grams per square meter (gsm) were produced.

In all cases the base sheets were produced from a furnish comprising northern softwood kraft and eucalyptus kraft using a layered headbox fed by three stock chests such that

the webs having three layers (two outer layers and a middle layer) were formed. The two outer layers comprised eucalyptus (each layer comprising 30 percent weight by total weight of the web) and the middle layer comprised softwood and eucalyptus. The amount of softwood and eucalyptus kraft in the middle layer was maintained for all inventive samples—the middle layered comprised 29 percent (by total weight of the web) softwood and 11 percent (by total weight of the web) eucalyptus. Strength was controlled via the addition of starch and/or by refining the furnish.

The tissue web was formed on a forming fabric, vacuum dewatered to approximately 25 percent consistency and then subjected to rush transfer when transferred to the transfer fabric. The web was then transferred to a through-air drying fabric. Transfer to the through-drying fabric was done using vacuum levels of about 10 inches of mercury at the transfer. The web was then dried to approximately 98 percent solids before winding. Table 1 summarizes the physical properties of the basesheet webs.

TABLE 1

| Sample      | BW (gsm) | GMT (g/3") | Caliper (mils) |
|-------------|----------|------------|----------------|
| Basesheet 1 | 46.0     | 1125       | 26.15          |
| Basesheet 2 | 46.0     | 1367       | 26.81          |
| Basesheet 3 | 42.2     | 798        | 19.2           |
| Basesheet 4 | 41.8     | 994        | 19.7           |

The inventive softening compositions were prepared by mixing the cationic softening compound with a small amount of water using a high shear mixer. After mixing, the polyhydroxy compound was added along with silicone, as specified in Table 2 below, followed by further high shear mixing. The pH of the composition was adjusted and the composition was further diluted with water and mixed. Viscosity was measured by Brookfield DV-II ultra-type (Brookfield Engineering Laboratories) at  $25^\circ\text{C}$ . and 60 rpm. The silicone was UTA6014 (Commercially available from Wacker Chemical Corp., Adrian, Mich.) and cationic softening compound was either CEQ90 (Commercially available from Sunjin Chemical Co. Ltd) (softener composition 1) or Incroquat Behenyl TMS-50, (commercially available from Croda Inc., Edison, N.J.) (softener composition 2).

TABLE 2

|                         | Softener Composition 1 | Softener Composition 2 |
|-------------------------|------------------------|------------------------|
| Silicone (wt %)         | 30                     | 30                     |
| Softener (wt %)         | 14                     | 7                      |
| PEG-1,000 (wt %)        | 7                      | 7                      |
| Water (wt %)            | 49                     | 60                     |
| Estimated % Solids      | 34                     | 27                     |
| Initial viscosity (cPs) | 140                    | 650                    |

The base sheet webs were converted into bath tissue rolls. Specifically, basesheet was calendered using a conventional polyurethane/steel calender system comprising a 40 P&J polyurethane roll on the air side of the sheet and a standard steel roll on the fabric side. The calendered web was then subjected to topical treatment with a softening composition. The softening compositions were applied by offset gravure printing. The add-on levels were controlled by changing the gravure roll cell volume (measured as BCM—billion cubic microns per square inch) and estimated add-on levels are reported in Table 3, below. The estimated add-ons are provided as both a wet weight basis and a dry weight percentage basis.

TABLE 3

| Sample      | Basesheet | Gravure roll cell volume (BCM) | Estimated Softening Composition Add-on (wet grams per square meter) | Estimated Softening Composition Add-on (dry wt %) |
|-------------|-----------|--------------------------------|---------------------------------------------------------------------|---------------------------------------------------|
| Control 1   | 1         | —                              | —                                                                   | —                                                 |
| Control 2   | 2         | —                              | —                                                                   | —                                                 |
| Inventive 1 | 1         | 4                              | 1.65                                                                | 1.3                                               |
| Inventive 2 | 2         | 4                              | 1.65                                                                | 1.3                                               |
| Inventive 3 | 1         | 6                              | 4.65                                                                | 3.5                                               |
| Inventive 4 | 2         | 6                              | 4.65                                                                | 3.5                                               |
| Inventive 5 | 3         | 6                              | 7.14                                                                | 4.4                                               |
| Inventive 6 | 4         | 6                              | 7.14                                                                | 4.4                                               |

The finished products were subjected to physical analysis, which is summarized in Tables 4 and 5, below.

TABLE 4

| Sample      | Softening Composition Add-on (dry wt %) | Basis Weight (gsm) | GMT (g/3") | Caliper (mils) | Sheet Bulk (cc/g) | MD COF (g) |
|-------------|-----------------------------------------|--------------------|------------|----------------|-------------------|------------|
| Control 1   | —                                       | 43.1               | 933        | 26.15          | 14.44             | 288        |
| Control 2   | —                                       | 43.6               | 1074       | 26.81          | 14.80             | 276        |
| Inventive 1 | 1.3                                     | 44.0               | 929        | 24.89          | 13.74             | 231        |
| Inventive 2 | 1.3                                     | 44.1               | 1099       | 25.46          | 14.06             | 207        |
| Inventive 3 | 3.5                                     | 44.4               | 922        | 25.67          | 14.17             | 213        |
| Inventive 4 | 3.5                                     | 44.9               | 1080       | 25.93          | 14.32             | 197        |
| Inventive 5 | 4.4                                     | 42.2               | 785        | 18.05          | 12.60             | 190        |
| Inventive 6 | 4.4                                     | 42.0               | 874        | 18.35          | 12.99             | 193        |

TABLE 5

| Sample      | CD Tensile (g/3") | CD Stretch (%) | CD TEA (g*cm/cm <sup>2</sup> ) | GM Slope (kg) | Stiffness Index |
|-------------|-------------------|----------------|--------------------------------|---------------|-----------------|
| Control 1   | 764               | 8.6            | 6.06                           | 6.801         | 7.29            |
| Control 2   | 877               | 9.0            | 7.45                           | 7.136         | 6.64            |
| Inventive 1 | 732               | 7.8            | 5.48                           | 7.474         | 8.05            |
| Inventive 2 | 851               | 8.4            | 6.65                           | 7.705         | 7.01            |
| Inventive 3 | 785               | 8.0            | 5.62                           | 7.689         | 8.34            |
| Inventive 4 | 840               | 8.0            | 6.39                           | 8.072         | 7.47            |
| Inventive 5 | 794               | 8.8            | 7.0                            | 5.712         | 7.27            |
| Inventive 6 | 1010              | 8.4            | 8.2                            | 5.827         | 6.66            |

While various softening compositions, and tissue webs and products treated therewith, have been described in detail with respect to the specific embodiments thereof, it will be appreciated that those skilled in the art, upon attaining an understanding of the foregoing, may readily conceive of alterations to, variations of, and equivalents to these embodiments. Accordingly, the scope of the present invention should be assessed as that of the appended claims and any equivalents thereto and the following embodiments.

In a first embodiment the present invention provides a treated through-air dried tissue product comprising a through-air dried tissue web having a first and an opposed second surface, a softening composition disposed on the first or the second surface, the softening composition comprising (i) a polyhydroxy compound having a molecular weight of at least about 1,000 g/mol and (ii) a cationic softener compound, the treated through-air dried tissue product having a COF less than about 300 g.

In a second embodiment the present invention provides the tissue product of the first embodiment having a COF less than about 250 g.

In a third embodiment the present invention provides the tissue product of the first or the second embodiments having a COF from about 200 to about 250 g, a GMT from about 700 to about 1,200 g/3" and a Stiffness Index less than about 10.

In a fourth embodiment the present invention provides the tissue product of any one of the first through third embodiments wherein the cationic softener compound selected from the group consisting of amidoamine quaternary ammonium compounds, diamidoamine quaternary ammonium compounds, ester quaternary ammonium compounds, alkoxy alkyl quaternary ammonium compounds, benzyl quaternary ammonium compounds, alkyl quaternary ammonium compounds and imidazolinium compounds.

In a fifth embodiment the present invention provides the tissue product of any one of the first through fourth embodiments wherein the softening composition further comprises a silicone, a glycerin, or mixtures thereof.

In a sixth embodiment the present invention provides the tissue product of any one of the first through fifth embodiments wherein the softening composition comprises less than about 12 dry weight percent, based upon the dry weight of the tissue product.

In a seventh embodiment the present invention provides the tissue product of any one of the first through sixth embodiments wherein the softening composition comprises from about 0.5 to about 5.0 dry weight percent, based upon the dry weight of the tissue product.

In an eighth embodiment the present invention provides the tissue product of any one of the first through seventh embodiments wherein the softening composition comprises from about 10 to about 20 weight percent of a cationic softening compound and from about 10 to about 20 weight percent of a polyhydroxy compound.

In a ninth embodiment the present invention provides the tissue product of any one of the first through eighth embodiments wherein the softening composition comprises from about 40 to about 75 weight percent water and the ratio of water to the polyhydroxy compound, on a weight basis, is from about 1:0.1 to about 1:10.

We claim:

1. A treated through-air dried tissue product comprising a through-air dried tissue web having a first and an opposed second surface, a softening composition disposed on the first or the second surface, the softening composition comprising (i) from about 10 to 20 weight percent of a polyhydroxy compound selected from the group consisting of polyethylene glycols and polypropylene glycols and having a molecular weight from about 1,000 to about 10,000 g/mol (ii) from about 10 to about 20 weight percent of a cationic softener compound selected from the group consisting of amidoamine quaternary ammonium compounds, diamidoamine quaternary ammonium compounds, ester quaternary ammonium compounds, alkoxy alkyl quaternary ammonium compounds, benzyl quaternary ammonium compounds, alkyl quaternary ammonium compounds and imidazolinium compounds, and (iii) from about 40 to about 75 weight percent water, the treated through-air dried tissue product having a coefficient of friction (COF) less than about 300 g.

2. The treated through-air dried tissue product of claim 1 having a sheet bulk greater than about 10 cc/g and a COF less than about 250 g.

3. The treated through-air dried tissue product of claim 1 further comprising a silicone, or a glycerin, and mixtures thereof.

## 19

4. The treated through-air dried tissue product of claim 1 wherein the softening composition comprises from about 0.5 to about 5.0 dry weight percent, based upon the dry weight of the tissue product.

5. The treated through-air dried tissue product of claim 1 wherein the weight ratio of cationic softener to polyhydroxy compound are from about 1:0.3 to about 0.3:1.

6. The treated through-air dried tissue product of claim 1 wherein the polyhydroxy compound is a polyethylene glycol having a molecular weight from about 4,000 to about 10,000 g/mol and the weight ratio of water to polyhydroxy compound are from about 1:02 to about 1:5.

7. The treated through-air dried tissue product of claim 1 further comprising less than about 2.0 weight percent silicone.

8. The treated through-air dried tissue product of claim 1 wherein the tissue product is substantially free from silicone.

9. The treated through-air dried tissue product of claim 1 wherein the softening composition comprises from about 10 to about 15 weight percent polyhydroxy compound.

10. The treated through-air dried tissue product of claim 9 wherein the polyhydroxy compound has a molecular weight from about 6,000 to about 8,000 and wherein the weight ratio of cationic softener to polyhydroxy compound is about 1:0.7 to about 0.7:1.

11. A treated through-air dried tissue product comprising a through-air dried tissue web having a first and an opposed second surface, a softening composition disposed on the first or the second surface, the softening composition comprising:

a. from about 10 to about 20 weight percent of a cationic softening compound selected from the group consisting of diamidoamine quaternary compounds, ester quaternary compounds, alkoxy alkyl quaternary compounds, benzyl quaternary compounds, alkyl quaternary compounds and imidazolinium quaternary compounds;

a. from about 10 to about 20 weight percent of a polyhydroxy compound selected from the group consisting of polyethylene glycols and polypropylene glycols having a molecular weight of at least about 1,000 g/mol;

b. from about 60 to about 80 percent water; and

c. optionally a silicone or glycerin,

wherein the treated tissue product has a coefficient of friction (COF) less than about 300 g.

12. The treated through-air dried tissue product of claim 11 having a GMT from about 500 to about 1,500 g/3", a Stiffness Index less than about 15 and a sheet bulk greater than about 10 cc/g.

## 20

13. The treated through-air dried tissue product of claim 11 wherein the softening composition comprises from about 0.5 to about 5.0 weight percent, based upon the dry weight of the tissue product.

14. The treated through-air dried tissue product of claim 11 wherein the softening composition comprises a polyethylene glycol having a molecular weight from about 1,000 to about 10,000.

15. The treated through-air dried tissue product of claim 11 wherein the ratio of water to the polyhydroxy compound, on a weight basis, is from about 1:0.1 to about 1:10.

16. A method of manufacturing a soft through-air dried tissue product comprising the steps of:

a. forming an aqueous softening composition comprising  
(i) from about 10 to 20 weight percent of a polyhydroxy compound selected from the group consisting of polyethylene glycols and polypropylene glycols and having a molecular weight from 1,000 to about 10,000 g/mol  
(ii) from about 10 to about 20 weight percent of a cationic softener compound selected from the group consisting of amidoamine quaternary ammonium compounds, diamidoamine quaternary ammonium compounds, ester quaternary ammonium compounds, alkoxy alkyl quaternary ammonium compounds, benzyl quaternary ammonium compounds, alkyl quaternary ammonium compounds and imidazolinium compounds, (iii) from about 40 to about 75 weight percent water, and optionally a silicone or glycerin;

b. providing a through-air dried tissue web having a first and an opposed second surface; and

c. applying the aqueous softening composition at a temperature less than about 100° C. to at least the first surface of the through-air dried tissue web.

17. The method of claim 16 wherein the through-air dried tissue web is a dry tissue web and the step of applying is carried out by slot coating, gravure printing, flexographic printing or spraying.

18. The method of claim 16 wherein the aqueous softening composition is applied at a temperature from about 20 to about 30° C.

19. The method of claim 16 wherein the aqueous softening composition comprises from about 30 to about 70 weight percent water and has a viscosity from about 50 to about 300 cPs.

\* \* \* \* \*